

## UNITED STATES PATENT OFFICE

FRANK RABAK, OF WASHINGTON, DISTRICT OF COLUMBIA, DEDICATED TO THE GOVERNMENT AND THE PEOPLE OF THE UNITED STATES OF AMERICA

PROCESS FOR COATING AND SEALING RED CEDAR LUMBER TO PREVENT THE ESCAPE OF CEDAR AROMA

No Drawing.

Application filed August 2, 1930. Serial No. 472,742.

(GRANTED UNDER THE ACT OF MARCH 3, 1883, AS AMENDED APRIL 30, 1928; 370 O. G. 757)

This application is made under the act approved April 30, 1928, and the invention herein described, if patented, may be manufactured and used by or for the Government for governmental purposes without payment to me of any royalty thereon. 5

I hereby dedicate the invention herein described to the free use of the public to take effect upon the granting of a patent to me. 10

The use of cedar, particularly red cedar, for the manufacture of containers for clothing, particularly cedar chests and cedar closets in homes, has come to be quite extensive because of the efficacy of the aroma in preventing moths from inhabiting and destroying or injuring articles of clothing stored in such containers. Because of the comparative scarcity of red cedar and the consequent cost of same, closets and chests for the purpose stated are now commonly lined with the red cedar wood and the manufacture and sale of cedar closet lining has come to be an industry of considerable proportions in this country. The red cedar is cut into boards or strips of appropriate thickness and with, say approximately  $\frac{1}{8}$ " in thickness by  $2\frac{1}{4}$ " in width with the edges formed to be interengaged by tongue-and-groove formation. 15

The efficiency of the red cedar for the purpose mentioned is dependent upon the maximum concentration of cedar aroma or vapor within the closet or chest. The aroma or vapor from the cedar is produced by volatilization of the essential oil contained in the wood. 20 As the result of experiments extending over a considerable period of time, I have discovered that when cedar boards are exposed to the air there is a loss of oil by volatilization, which loss is proportionate to the thickness of the boards and the length of time exposed. Cedar boards exhale aroma and thereby lose oil from all exposed surfaces. 25 As will be readily understood the aroma exhaled from the exterior surface of the board is lost. In order to conserve the volatile oil it is important that loss from such exterior surfaces be prevented. In cedar chests this is sometimes in a measure accomplished by the finishing coating on the exterior of the cedar. In cedar closets, how-

ever, which are constructed by boarding up the side walls and ceiling with the cedar boards attached directly to the studs and joists such loss from the exterior surfaces is material and all waste, with the resulting efficiency of the closet for the purposes intended greatly depreciated. 55

Since the cedar boards exhale aroma from all exposed surfaces it will be readily understood that the exterior surface gives off the aroma in the same volume as the interior surface. The aroma volatilized from the exterior of the boards is practically lost to the interior of the closet. For the purpose of conserving the aroma and prolonging the efficiency of the closet, chest or other container lined with the cedar, these experiments have been conducted to discover a material suitable to apply to the surfaces of the board which it is desired to seal against the escape of the aroma and the best and most practical method of application. In planning the procedure for the experiments several important points were regarded as entitled to particular consideration as follows: 60 65 70 75

(1) Effective sealing of the exterior to prevent any escape of oil (cedar aroma) in that direction.

(2) A coating that would be transparent and with no covering power in order that it could be observed by a glance that the boards were of red heart wood only, the type of wood recognized as most efficient for the purpose. 80

(3) A coating that should permit of easy application and dry quickly and permanently. 85

(4) A coating that after being applied to the boards should be free from all stickiness or tackiness in order that the boards might be packed in bundles without adhering to each other, as in making up packages for shipment and handling as an article of commerce. 90

(5) Low cost of the material and of the application of the same to the boards. 95

In order to effectively seal the wood to prevent the escape of the oil, the coating must necessarily be of such nature that the thin film on the wood should be insoluble in the oil of the cedar or in the cedar vapors. Also, 100

it should combine transparency and rapid drying qualities, lack of stickiness and low cost.

The following materials have been used in my experiments:

5 *Orange shellac*.—A varnish prepared by dissolving orange shellac in denatured alcohol. A commercial product obtainable in the open market.

10 *Lacquer (clear)*.—Obtainable in the market as brushing lacquers (clear).

*Floor varnish (4 hr.)*.—A special type of floor varnish which dries to extreme hardness in four hours; obtainable on the market.

15 *Paraffin (M. P. 55° C.)*.—Prepared by dissolving three pounds of paraffin in one gallon of an appropriate vehicle, as for example, carbon tetrachloride or gasoline.

20 *Gum arabic*.—A 20 per cent solution of commercial powdered gum arabic in water.

*Gelatin*.—A 10 per cent solution of commercial crude gelatin in water.

25 *Water-glass (sodium silicate)*.—Commercial sirupy water-glass diluted in the proportion of 250 parts of water-glass to 25 parts of water.

For use in making the desired tests, miniature tight cedar closets, or boxes (4 in. by 8 in. by 12 in.) with a hinged lid, were constructed 30 of  $\frac{1}{2}$  inch red cedar heart wood. The coatings were applied to the exterior of the boxes as uniformly as possible by means of a flat varnish brush. The coated boxes together with an uncoated box as a check were set aside and kept in a warm room for a period 35 of several months, after which a careful examination of each was made.

Examination of the boxes after such exposure at temperatures between 70° and 90°

40 F. showed that all the coatings effectively sealed the wood and prevented the escape of the cedar oil, no odor of cedar being perceptible on the outside of the boxes. The interior of the boxes had an unusually strong

45 odor of cedar. The check box with no coating had a distinct odor of cedar which indicated that the wood was still exhaling odor into the atmosphere.

Since the appearance of the wood after the 50 application of the coatings has an important bearing on the practicability of the various materials used, a careful analysis of the appearance in each instance was made.

The box coated with paraffin seemed the 55 most natural in appearance, the red color of the cedar apparently being unchanged; also there was a total absence of gloss.

The boxes coated with gum arabic and gelatine, respectively, were also practically 60 unchanged in color but both were slightly glossy.

The lacquer-coated box preserved the original red color to a marked degree with only very slight gloss apparent.

65 *Orange shellac* slightly intensified the red

color and imparted a slight glossy appearance to the wood.

*Floor varnish* darkened the original red color and produced a distinct gloss.

70 *Water-glass* caused a change of the red color to a pale dirty brown and the box was distinctly glossy.

75 The quick drying lacquer, orange shellac and paraffin excelled the other coatings, drying almost immediately to a non-tacky condition. *Floor varnish* required approximately four hours to dry non-tacky, while gum arabic, gelatine and water-glass, being aqueous solutions, dried by evaporation of the moisture in from 1 to 2 hours.

80 An approximate estimate of the cost of these materials was made, based on the current wholesale price of the materials used. The cost of application was not estimated because of the fact that by mechanical means, such as would be used on a factory scale, it would be considerably less than application by hand.

85 *Paraffin, lacquer, orange shellac and floor varnish* are most effectively and economically applied by spraying or atomizing, while the other coatings could probably be less satisfactorily applied in this manner.

90 From the experiments with these materials extending over a period of time, I have selected paraffin as the coating especially desirable for the purpose. While I advocate the use of paraffin I do not wish to be restricted to its use alone. Paraffin has the advantage over other materials because of its low cost, and the desirable feature of effectiveness, quick drying and non-sticky qualities, without changing, obscuring or hiding the color of the original wood.

95 The "non-sticky" quality of the coating is very important because of the fact that the boards are put up for sale in packages of practically airtight character and oftentimes remain in these packages for many months. Under these circumstances many of the coatings which otherwise would be reasonably practicable become impracticable on account of their tendency to become sticky and cause the boards to stick together in the package, injuring or destroying their value for the purposes for which they are designed. When dissolved in carbon tetrachloride the hazard in its application due to inflammability is overcome.

100 *Orange shellac* possesses rapidity of drying and ease of application by the spraying method. It does not materially alter the appearance of the wood and is an effective coating obtainable at relatively low cost.

105 *Lacquer (clear)* is ideal in all respects as a coating but is higher in cost. This, however, is probably not prohibitive.

110 The choice of coating can best be determined by the manufacturer and doubtless would depend largely on the cost which, how-

ever, should be more than offset by the superior quality and effectiveness of the cedar lining for the purpose.

Having thus fully described my said invention, what I claim as new and desire to secure by Letters Patent, is:

1. A lining for containers such as closets and chests consisting of cedar boards one surface of which is coated with a transparent sealing substance comprising paraffin which substance is adapted to seal the pores of the wood against the escape of the volatile oil or aroma but at the same time leave the wood surface exposed to view, and the other surface of which is left uncoated whereby the volatile oil or aroma of the cedar may escape freely into the interior of containers lined therewith.

2. A closed receptacle lined with cedar boards the face of the lining boards next to the walls of the receptacle being coated with a transparent non-adhesive sealing substance comprising paraffin to prevent the escape through such side of the volatile oils or aroma of the cedar, and the inner face of such lining boards being left uncoated, whereby the volatile oil or aroma of the cedar may escape freely into the interior of the receptacle.

FRANK RABAK.

30

35

40

45

50

55

60

65